

# UNITED STATES PATENT OFFICE.

PAUL RICHARD KUEHNRICH, OF SHEFFIELD, ENGLAND.

## MANUFACTURE OF STEEL.

No Drawing.

Application filed June 28, 1923. Serial No. 648,358.

*To all whom it may concern:*

Be it known that I, PAUL RICHARD KUEHNRICH, a subject of the King of England, residing at Sheffield, in Yorkshire, England, have invented certain new and useful Improvements in or Relating to the Manufacture of Steel (for which I filed an application for patent in Great Britain on the 1st July, 1922, No. 18,105); and I do hereby declare that the following is a full, clear, and exact description of the same.

This invention relates to the manufacture of steel, its object being to provide an improved cementation process by diffusion of the hardening constituents.

The process according to the present invention is carried out in a fused salt bath and comprises the simultaneous diffusion of the three elements, boron, carbon and nitrogen. The articles to be treated are manufactured from iron or steel of the desired composition but with a lower percentage of carbon than is or would normally be required in the finished state. They are suspended in a bath of fused salts, the bulk of which consists of a relatively inert salt (or mixture) such as barium chloride or calcium chloride of the kind generally used for the heat treatment of steel. According to the present invention, however, hardening properties are imparted to the iron or steel by adding to this relatively inert salt proportions of other fusible salts containing boron, carbon and nitrogen. Different salts in which one or more of these three elements are combined may be used according to circumstances and their proportions may vary. For example to provide mild steel (0.15 carbon) articles with a skin which may be hardened sufficiently to scratch glass a bath may be used consisting of 95% of barium chloride and 5% of calcium borate, potassium carbonate and potassium ferro-cyanide or potassium cyanide in equal proportions by weight.

It appears that the boron first penetrates

the article treated and acts as a catalyst for the diffusion of the carbon and nitrogen. Articles treated according to the present invention may be hardened, annealed and re-hardened.

The bath is preferably heated by electrical means, but other sources of heat such as gas or coke may be used, and it is found that articles suspended or immersed in the mixture of fused salts according to this invention are converted very much more rapidly than by any known cementation process. In addition to the case-hardening effect, a diffusion and conversion to a very much greater depth also takes place.

What I claim is:—

1. The method of imparting hardening properties to iron or steel by suspending it in a bath of fused salts the bulk of which is relatively inert and is mixed with a proportion of other fusible salts containing boron, carbon and nitrogen, substantially as specified.

2. The method of imparting hardening properties to iron or steel by suspending it in a bath of fused salts consisting of about 95% of barium chloride and of about 5% of calcium borate, potassium carbonate and potassium ferro-cyanide or potassium cyanide in substantially equal proportions, substantially as specified.

3. The method of imparting hardening properties to iron or steel by suspending it in a bath of fused salts consisting of about 95% of a mixture of barium chloride and calcium chloride and of about 5% of calcium borate, potassium carbonate and potassium ferro-cyanide or potassium cyanide in substantially equal proportions, substantially as specified.

In testimony whereof I hereunto affix my signature.

PAUL RICHARD KUEHNRICH.

Witnesses:

ARTHUR H. GREENWOOD,  
HAWTHORN ULRIGHT.